



US008182971B2

(12) **United States Patent**  
**Koike et al.**

(10) **Patent No.:** **US 8,182,971 B2**  
(45) **Date of Patent:** **May 22, 2012**

(54) **RESIN FOR TONER AND TONER COMPOSITION**

(75) Inventors: **Masanori Koike**, Kyoto (JP); **Yasuhiro Ono**, Kyoto (JP)

(73) Assignee: **Sanyo Chemical Industries, Ltd.**, Kyoto (JP)

(\*) Notice: Subject to any disclaimer, the term of this patent is extended or adjusted under 35 U.S.C. 154(b) by 590 days.

(21) Appl. No.: **11/921,134**

(22) PCT Filed: **May 26, 2006**

(86) PCT No.: **PCT/JP2006/310531**

§ 371 (c)(1),  
(2), (4) Date: **Aug. 10, 2009**

(87) PCT Pub. No.: **WO2006/126667**

PCT Pub. Date: **Nov. 30, 2006**

(65) **Prior Publication Data**

US 2009/0305157 A1 Dec. 10, 2009

(30) **Foreign Application Priority Data**

May 27, 2005 (JP) ..... 2005-155182

(51) **Int. Cl.**  
**G03G 9/00** (2006.01)

(52) **U.S. Cl.** ..... **430/109.4**; 525/418; 528/271;  
528/272; 528/296

(58) **Field of Classification Search** ..... 430/109.4;  
525/418; 528/271, 272, 296

See application file for complete search history.

(56) **References Cited**

U.S. PATENT DOCUMENTS

4,960,664 A 10/1990 Yamada et al.  
5,830,979 A 11/1998 Nakayama et al.  
2001/0051309 A1 \* 12/2001 Nagahama et al. ..... 430/108.23

FOREIGN PATENT DOCUMENTS

|    |             |         |
|----|-------------|---------|
| EP | 1 186 962   | 3/2002  |
| GB | 2 289 950   | 12/1995 |
| JP | 05-080586   | 4/1993  |
| JP | 06-027728   | 2/1994  |
| JP | 09-251216   | 9/1997  |
| JP | 11-153884   | 6/1999  |
| JP | 11-249339   | 9/1999  |
| JP | 2000-321819 | 11/2000 |
| JP | 2001-125307 | 5/2001  |
| JP | 2002-318471 | 10/2002 |
| JP | 2004-184561 | 7/2004  |
| JP | 2004-271859 | 9/2004  |
| JP | 2005-062517 | 3/2005  |
| JP | 2005-128122 | 5/2005  |

OTHER PUBLICATIONS

Extended European Search Report mailed Jun. 24, 2011, in corresponding European Patent Application No. 06756631.5.

Notification of Reason for Refusal dated Sep. 28, 2010, in corresponding Japanese Patent Application No. 2006-146389 (with English translation).

International Search Report for PCT/JP2006/310531.

\* cited by examiner

*Primary Examiner* — Mark A Chapman

(74) *Attorney, Agent, or Firm* — Edwards Wildman Palmer LLP

(57) **ABSTRACT**

A toner and a resin for toner are provided which are of good low-temperature fixing ability and good anti-blocking property of toner at high temperature and high humidity and good pulverisability. The present invention is directed to a resin for toner, the resin comprising a polyester resin (A) produced by reacting a polyester resin (a) having an acid value of 6 mgKOH/g or less and a hydroxyl value of 10 to 80 mgKOH/g with at least one carboxylic acid (b) selected from the group consisting of aliphatic carboxylic acids, aromatic carboxylic acids, their anhydrides and lower alkyl (C1-C4) esters, wherein the equivalent ratio OH<sub>a</sub>/COOH<sub>b</sub> is 0.55 to 1.0 where OH<sub>a</sub> represents the equivalent of the hydroxyl groups originating in (a) in the reaction of (a) and (b) and COOH<sub>b</sub> represents the equivalent of the carboxyl groups originating in (b) in the reaction of (a) and (b), and wherein the polyester resin (A) has an acid value of 13 to 50 mgKOH/g and a hydroxyl value of 8 mgKOH/g or less; and a toner composition including the same.

**12 Claims, No Drawings**

## 1

## RESIN FOR TONER AND TONER COMPOSITION

## CROSS-REFERENCE TO RELATED APPLICATIONS

This application is the 35 U.S.C. §371 national stage of PCT application PCT/JP2006/310531, filed May. 26, 2006, which claims priority to Japanese patent application No. 2005-155182, filed May. 27, 2005. The contents of these applications are incorporated herein by reference in their entirety.

## TECHNICAL FIELD

The present invention relates to resins for toners and toner compositions to be used in electrophotography, electrostatic recording, electrostatic printing and so on.

## BACKGROUND ART

Use of a polyester resin as a binder for improving the low-temperature fixing ability of a toner is known (see, for example, patent documents 1, 2). An approach of incorporating a crystalline resin is also proposed for improvement in low-temperature fixing ability (see, for example, patent documents 3).

Patent document 1: JP 62-78568 A

Patent document 2: JP 62-178278 A

Patent document 3: JP 2003-337443 A

## DISCLOSURE OF THE INVENTION

## Problem to Be Solved by the Invention

Reduction in molecular weight is needed in order to further improve the low-temperature fixing ability of a toner. In such cases, however, there is a problem that toners are somewhat poor in anti-blocking property at high temperature and high humidity. In addition, incorporation of a crystalline resin has a problem of affecting pulverisability.

## Means for Solving the Problem

The inventors of the present invention studied assiduously to solve such problems and, as a result, have reached the invention.

That is, the invention provides: [1] a resin for toner, the resin comprising a polyester resin (A) produced by reacting a polyester resin (a) having an acid value of 6 mgKOH/g or less and a hydroxyl value of 10 to 80 mgKOH/g with at least one carboxylic acid (b) selected from the group consisting of aliphatic carboxylic acids, aromatic carboxylic acids, their anhydrides and lower alkyl (C1-C4) esters, wherein the equivalent ratio OH<sub>a</sub>/COOH<sub>b</sub> is 0.55 to 1.0 where OH<sub>a</sub> represents the equivalent of the hydroxyl groups originating in (a) in the reaction of (a) and (b) and COOH<sub>b</sub> represents the equivalent of the carboxyl groups originating in (b) in the reaction of (a) and (b), and wherein the polyester resin (A) has an acid value of 13 to 50 mgKOH/g and a hydroxyl value of 8 mgKOH/g or less; [2] a resin for toner, the resin comprising a polyester resin (A') which has an acid value of 13 to 50 mgKOH/g and a hydroxyl value of 8 mgKOH/g or less and has a THF-insoluble matter in a content of 1 to 50% by weight, wherein 30 to 100 mol % of the polyol component constituting the (A') is an aliphatic diol having 2 to 6 carbon atoms and the carboxylic acid component constituting the

## 2

(A') comprises a trivalent or higher valent polycarboxylic acid; and [3] a toner composition comprising one of the above mentioned resins for toner, a colorant and, if necessary, one or more additives selected from mold release agents, charge control agents and fluidizing agents.

## Effect of the Invention

By use of the resin for toner of the present invention, a toner with excellent low-temperature fixing ability can be obtained and the anti-blocking property of the toner is also good. Further, toners can be produced economically in industrial manufacture because the resin shows excellent pulverisability during the toner production.

## BEST MODE FOR CARRYING OUT THE INVENTION

The invention will be described in detail.

20 The resin for toner of the present invention comprises a polyester resin (A) produced by reacting a polyester resin (a) having a specific acid value and a specific hydroxyl value with at least one carboxylic acid (b) selected from the group consisting of aliphatic carboxylic acids, aromatic carboxylic acids, their anhydrides and lower alkyl (C1-C4) esters.

25 As the polyester resin (a), preferred is a polyester resin obtained by polycondensing at least one polyol component with at least one polycarboxylic acid component.

It is preferred, in view of storage stability, that 30 to 100 30 mol %, more preferably 40 to 100 mol %, particularly preferably 50 to 100 mol %, and most preferably 80 to 100 mol % of the polyol component is an aliphatic diol having 2 to 6 carbon atoms. Because the polyester resin (A) is obtained by reacting a polyester resin (a) with a carboxylic acid (b), it is 35 preferred that the polyol component constituting the (A) is also that mentioned above.

40 Examples of aliphatic diols having 2 to 6 carbon atoms include alkanediols such as ethylene glycol, 1,2-propylene glycol, 1,3-propylene glycol, 1,4-butanediol, 2,3-butanediol, 1,5-pentanediol, 2,3-pentanediol, 1,6-hexanediol, 2,3-hexanediol, 3,4-hexanediol and neopentyl glycol. Two or more species may be used in combination. Preferred among them are ethylene glycol, 1,2-propylene glycol and neopentyl glycol. More preferred are ethylene glycol and 1,2-propylene glycol. Particularly preferred is 1,2-propylene glycol.

45 Examples of dihydric alcohol (diol) among polyol components other than aliphatic diols having 2 to 6 carbon atoms include aliphatic diols having 7 to 36 carbon atoms (1,7-heptanediol, dodecanediol, etc.); polyalkylene ether glycols having 4 to 36 carbon atoms (diethylene glycol, dipropylene glycol, polyethylene glycol, polypropylene glycol, etc.); adducts of aliphatic diols having 2 to 36 carbon atoms with alkylene oxides (herein after abbreviated as AO) having 2 to 4 carbon atoms [ethylene oxide (herein after abbreviated as EO), propylene oxide (herein after abbreviated as PO), butylene oxide, etc.] (additional molar number: 2 to 30); alicyclic diols having 6 to 36 carbon atoms (1,4-cyclohexanedimethanol, hydrogenated bisphenol A, etc.); adducts of the alicyclic diols with AOs having 2 to 4 carbon atoms (additional molar number: 2 to 30); and adducts of bisphenols (bisphenol A, bisphenol F, bisphenol S, etc.) with AOs having 2 to 4 carbon atoms (additional molar number: 2 to 30). Two or more species may also be used in combination.

55 Examples of tri- to octahydric or higher hydric polyols among polyol components include tri- to octahydric or higher hydric aliphatic polyols having 3 to 36 carbon atoms (glycerol, triethylolethane, trimethylolpropane, pentaerythritol,

sorbitol, etc.); adducts of the alicyclic polyols with AOs having 2 to 4 carbon atoms (additional molar number: 2 to 30); adducts of trisphenols (trisphenol PA, etc.) with AOs having 2 to 4 carbon atoms (additional molar number: 2 to 30); and adducts of novolak resins (phenol novolak, cresol novolak, etc.; average degree of polymerization: 3 to 60) with AOs having 2 to 4 carbon atoms (additional molar number: 2 to 30). Two or more species may be used in combination.

Preferred among such polyol components other than aliphatic diols having 2 to 6 carbon atoms are polyalkylene ether glycols having 4 to 36 carbon atoms, alicyclic diols having 6 to 36 carbon atoms, adducts of alicyclic diols having 6 to 36 carbon atoms with AOs having 2 to 4 carbon atoms, adducts of bisphenols with AOs having 2 to 4 carbon atoms, and adducts of novolak resins with AOs having 2 to 4 carbon atoms. More preferred are adducts of bisphenols with AOs having 2 to 3 carbon atoms (EO and/or PO) and adducts of novolak resins with AOs having 2 to 3 carbon atoms (EO and/or PO).

Aliphatic dicarboxyli acids (including alicyclic ones) among polycarboxylic acid components may be alkanedicarboxylic acids having 2 to 50 carbon atoms (oxalic acid, malonic acid, succinic acid, adipic acid, lepargylic acid, sebasic acid, etc.); and alkenedicarboxylic acids having 4 to 50 carbon atoms (alkenylsuccinic acids such as dodecenylnsuccinic acid, maleic acid, fumaric acid, citraconic acid, mesaconic acid, itaconic acid, glutaconic acid, etc.)

Aromatic dicarboxylic acids include, for example, aromatic dicarboxylic acids having 8 to 36 carbon atoms (phthalic acid, isophthalic acid, terephthalic acid, naphthalene-dicarboxylic acid, etc.).

Tri- or hexavalent or higher valent aliphatic polycarboxylic acids (including alicyclic ones) include, for example, aliphatic tricarboxylic acids having 6 to 36 carbon atoms (hexane tricarboxylic acid, etc.), and vinyl polymers of unsaturated carboxylic acids [number average molecular weight (herein after referred to as Mn, determined by gel permeation chromatography (GPC)): 450 to 10000] ( $\alpha$ -olefin-maleic acid copolymers, etc.).

Among polycarboxylic acid components, tri- to hexavalent or higher valent aromatic polycarboxylic acids include, for example, aromatic polycarboxylic acids having 9 to 20 carbon atoms (trimellitic acid, pyromellitic acid, etc.); vinyl polymers of unsaturated carboxylic acids [Mn: 450 to 10000] (styrene/maleic acid copolymer, styrene/acrylic acid copolymer, styrene/fumaric acid copolymer, etc.).

As a polycarboxylic acid component, anhydrides and lower (C1-C4) alkylesters (methylester, ethylester, isopropylester, etc.) of those polycarboxylic acids may also be used.

Preferred among such polycarboxylic acid components are alkane dicarboxylic acids having 2 to 50 carbon atoms, alkene dicarboxylic acids having 4 to 50 carbon atoms, aromatic dicarboxylic acids having 8 to 20 carbon atoms, and aromatic polycarboxylic acids having 9 to 20 carbon atoms. More preferred are adipic acid, alkenylsuccinic acids having 16 to 50 carbon atoms, terephthalic acid, isophthalic acid, maleic acid, fumaric acid, trimellitic acid, pyromellitic acid, and their combinations. Particularly preferred are adipic acid, terephthalic acid, trimellitic acid, and their combinations. Anhydrides and lower alkyl esters of these acids are also preferred.

A preferred example of the polycarboxylic acid component is one comprising an aromatic polycarboxylic acid and an aliphatic polycarboxylic acid and containing the aromatic polycarboxylic acid in an amount of 60 mol % or more. The content of the aromatic polycarboxylic acid is more preferably 70 to 99 mol %, and most preferably 80 to 98 mol %.

When an aromatic polycarboxylic acid is contained in an amount of 60 mol % or more, the resin strength increases and the low-temperature fixing ability is further improved.

In the present invention, the polyester resin (a) can be produced in a similar manner as the production method of conventional polyester. For example, it can be produced by carrying out a reaction under an inert gas atmosphere (nitrogen gas etc.), preferably at a reaction temperature of 150 to 280°C., more preferably 160 to 250°C., and most preferably 170 to 235°C. From the viewpoint of certain execution of a polycondensation reaction, the reaction time is preferably not less than 30 minutes, and particularly preferably 2 to 40 hours.

At this time, an esterification catalyst may also be used according to demand. Examples of the esterification catalyst include tin-containing catalysts (e.g., dibutyltin oxide), antimony trioxide, titanium-containing catalysts [e.g., titanium alkoxides, potassium titanyl oxalate, titanium terephthalate, titanium terephthalate alkoxide, and dihydroxybis(triethanolaminato) titanium and its intramolecular polycondensates], zirconium-containing catalysts (e.g., zirconium acetate), and zinc acetate. To improve the reaction rate of the last reaction stage, reducing the pressure is also effective.

The polyol component-to-polycarboxylic acid component reaction ratio, as expressed in terms of hydroxyl group-to-carboxyl group equivalent ratio [OH]/[COOH], is preferably 1.5/1 to 1/1, more preferably 1.2/1 to 1/1, and most preferably 1.1/1 to 1/1. When some component is removed out of the system during the reaction, the above-mentioned reaction ratio is a ratio calculated by excluding the component.

The polyester resin (a) has an acid value of 6 (mgKOH/g, in which the following acid values are also expressed) or less and a hydroxyl value of 10 to 80 (mgKOH/g, in which the following hydroxyl values are also expressed). The acid value is preferably 5 or less, and more preferably 4 or less. The hydroxyl value is preferably 15 to 65, and more preferably 20 to 58. If the acid value is greater than 6, or if the hydroxyl value is greater than 80, this means that the polyester resin (a) has been polycondensed insufficiently and it is rich in low molecular weight components and thus the storage stability worsens. If the hydroxyl value is smaller than 10, the reaction efficiency with the carboxylic acid (b) worsens.

In order to make the acid value and the hydroxyl value of a polyester resin (a) within those ranges, it is effective to adjust the reaction ratio of the polyol component with the polycarboxylic acid component.

The acid value and the hydroxyl value of a polyester resin referred to in the above and subsequent descriptions are determined by the methods provided in JIS K 0070 (1992).

In addition, in the case where a sample contained a solvent-insoluble component caused by crosslinking, a sample after melt kneaded is used in the following method.

Kneading apparatus: Labo plastomill MODEL 30R150 manufactured by Toyo Seiki Seisaku-sho, Ltd.

Kneading conditions: at 130°C., 70 rpm for 30 minutes

Regarding the molecular weight of the polyester resin (a), the peak top molecular weight (herein after, Mp) is preferably 2000 to 10000. It is more preferable that the Mp is 2500 to 9000.

In the above and following descriptions, the molecular weights (Mp and Mn) of a polyester resin are determined using GPC under the following conditions.

Apparatus (example): HLC-8120, manufactured by Tosoh Corp.

Column (example): TSK GEL GMH6 (two columns), manufactured by Tosoh Corp.

## 5

Measuring temperature: 40° C.

Sample solution: 0.25% by weight THF solution

Solution injection amount: 100  $\mu$ l

Detection apparatus: Refractive index detector

Reference material: Standard polystyrenes produced by Tosoh Corp. (TSK standard POLYSTYRENE) 12 points (Mw 1050, 2800, 5970, 9100, 18100, 37900, 96400, 190000, 355000, 1090000, 2890000 and 4480000)

The molecular weight corresponding to the maximum peak height on the chromatogram obtained is referred to as "peak top molecular weight (Mp)". In the measurement of the molecular weight of resin particles for toner, a solution prepared by picking up one arbitrary particle in a polyester resin for toner, dissolving it in THF and removing insoluble matters with a glass filter was used as a sample solution. This measurement was carried out for 10 particles.

The polyester resin (A) is obtained by causing a polyester resin (a) and a carboxylic acid (b) to react at a mixing ratio in the reaction expressed by an equivalent ratio OH<sub>a</sub>/COOH<sub>b</sub> of 0.55 to 1.0, where the equivalent of the hydroxyl groups originating in (a) is represented by OH<sub>a</sub> and the equivalent of the carboxyl groups originating in (b) is represented by COOH<sub>b</sub>. The OH<sub>a</sub>/COOH<sub>b</sub> is preferably 0.58 to 0.9, and more preferably 0.6 to 0.85. When the OH<sub>a</sub>/COOH<sub>b</sub> is less than 0.55, the molecular weight does not increase sufficiently and, therefore, the hot offset resistance of the toner compounding therefrom will deteriorate. When the ratio is greater than 1.0, the fluidity of the resin is reduced and, as a result, the low-temperature fixing ability of the toner compounding therefrom will deteriorate.

As the carboxylic acid (b), any one or both a monocarboxylic acid and a polycarboxylic acid may be used. Regarding the ratio of the monocarboxylic acid to the polycarboxylic acid, the equivalent ratio of the carboxyl groups originating in the monocarboxylic acid to the carboxyl groups originating in the polycarboxylic acid is preferably (0-50)/(50-100), and more preferably (0-20)/(80-100), where the equivalence of all the carboxyl groups in the carboxylic acids used in the reaction is considered to be 100. When the ratio of the carboxyl groups originating in the monocarboxylic acid is 50 or less, crosslinking does not occur insufficiently and the resin will become strong enough. Further, it is easy to adjust the acid value of a reaction product in a predetermined range easily.

As the carboxylic acid component, acid anhydrides and lower (C1-C4) alkylesters (methylester, ethylester, isopropyl ester, etc.) may also be used.

Among the monocarboxylic acids to be used as the carboxylic acid (b), examples of aliphatic (including alicyclic) monocarboxylic acids include alkane monocarboxylic acids having 1 to 50 carbon atoms (formic acid, acetic acid, propionic acid, butanoic acid, isobutanoic acid, caprylic acid, capric acid, lauric acid, myristic acid, palmitic acid, stearic acid, etc.), and alkene monocarboxylic acids having 3 to 50 carbon atoms (acrylic acid, methacrylic acid, oleic acid, linoleic acid, etc.).

The aromatic monocarboxylic acids include, for example, aromatic monocarboxylic acids having 7 to 36 carbon atoms (benzoic acid, methylbenzoic acid, phenylpropionic acid, naphthoic acid, etc.).

Among the polycarboxylic acids to be used as (b), examples of aliphatic (including alicyclic) dicarboxylic acid, aromatic dicarboxylic acids, tri-to hexavalent or higher valent aliphatic (including alicyclic) polycarboxylic acids, and tri-to hexavalent or higher valent aromatic polycarboxylic acids may be the same as those used in the polyester resin (a).

Preferred among these are divalent or higher valent aromatic carboxylic acids. More preferred are tri- to hexavalent

## 6

or higher valent aromatic polycarboxylic acids. Particularly preferred are trimellitic acid and trimellitic anhydride.

The polyester resin (A) can be obtained in the same production method as the polyester resin (a) except for adjusting the product to have an acid value and a hydroxyl value in the ranges given below.

The acid value of (A) is 13 to 50, and preferably 15 to 40. The hydroxyl value is 8 or less, and preferably not more than 6.

10 If the acid value is less than 13, the fixing strength becomes weak. If the hydroxyl value exceeds 8 or if the acid value exceeds 50, the product becomes susceptible to environmental conditions and the stability is deteriorated.

The THF-insoluble matter content of the polyester resin 15 (A) is preferably 1 to 50% by weight, and more preferably 2 to 35% by weight. If the THF-insoluble matter content is 1% by weight or more, good hot offset resistance is obtained and, if it is 50% by weight or less, the low-temperature fixing ability is good.

20 In the above and the following descriptions, a THF-insoluble matter content of a polyester resin is determined by the following method.

25 50 ml of THF was added to 0.5 g of a sample, and subjected to agitation under refluxing for three hours. After cooling, an insoluble component was filtered by a glass filter and the resin component remaining on the glass filter is subjected to drying under reduced pressure at 80° C. for three hours. An insoluble matter content is calculated from the ratio of the weight of the dried resin component on the glass filter and the weight of the 30 sample used.

35 Regarding the molecular weight of the polyester resin (A), Mp is preferably 4500 to 15000, and more preferably 5000 to 12000. Among polyester resins obtainable by a production method the same that of the resin of the first invention, a polyester resin (A') which has an acid value of 13 to 50 mgKOH/g and a hydroxyl value of 8 mgKOH/g or less and has a THF-insoluble matter in a content of 1 to 50% by weight, wherein 30 to 100 mol % (preferably, 80 to 100 mol %) of the polyol component constituting it is an aliphatic diol having 2 to 6 carbon atoms (preferably, 1,2-propylene glycol) and the carboxylic acid component constituting it comprises a trivalent or higher valent aromatic polycarboxylic acid is particularly suitable as a resin for toner (second invention) because the trivalent or higher valent aromatic carboxylic acid serves as a crosslinking agent to produce a sufficient resin strength.

40 45 The content of the trivalent or higher valent aromatic polycarboxylic acid in the carboxylic acid component is preferably 1 to 30 mol %, and more preferably 2 to 20 mol %. When the content is 30 mol % or less, the fluidity of the resin is good and, as a result, the low-temperature fixing ability of the toner compounding therefrom will be improved.

50 55 The composition and preferable substances of the raw materials for constituting the polyester resin (A'), the molecular weight of (A'), and the preferable ranges of the acid value, hydroxyl value and THF-insoluble matter content of (A') are the same as those of the polyester resin (A).

The resin for toner of the present invention may contain, together with the polyester resin (A), a polyester resin (B) other than the (A) which is free from any THF-insoluble matter. The term "polyester resin (A)" is hereafter used in a meaning encompassing the polyester resin (A').

60 65 The polyester resin (B) is typically obtained by polycondensing at least one polyol component with at least one polycarboxylic acid component.

Diols among the polyol components include, for example, aliphatic diols having 2 to 6 carbon atoms, aliphatic diols

having 7 to 36 carbon atoms, polyalkylene ether glycols having 4 to 36 carbon atoms, adducts of aliphatic diols having 2 to 36 carbon atoms with AOs having 2 to 4 carbon atoms (addition molar number: 2 to 30); alicyclic diols having 6 to 36 carbon atoms, adducts of alicyclic diols having 6 to 36 carbon atoms with AOs having 2 to 4 carbon atoms (addition molar number: 2 to 30); and adducts of bisphenols with AOs having 2 to 4 carbon atoms (addition molar number: 2 to 30). Two or more species may be used in combination. Specific examples of these materials may be the same as those to be used for the above-mentioned polyester resin (a).

Tri- to octahydric or higher hydric alcohols among the polyol components include, for example, tri- to octahydric or higher hydric aliphatic polyols having 3 to 36 carbon atoms, adducts of aliphatic polyols with AOs having 2 to 4 carbon atoms (addition molar number: 2 to 30); adducts of trisphenols with AOs having 2 to 4 carbon atoms (addition molar number: 2 to 30); and adducts of novolak resins with AOs having 2 to 4 carbon atoms (addition molar number: 2 to 30). Two or more species may be used in combination. Specific examples of these materials may be the same as those to be used for the above-mentioned polyester resin (a).

Preferred among such polyol components are aliphatic diols having 2 to 6 carbon atoms, polyalkylene ether glycols having 4 to 36 carbon atoms, alicyclic diols having 6 to 36 carbon atoms, adducts of alicyclic diols having 6 to 36 carbon atoms with AOs having 2 to 4 carbon atoms, adducts of bisphenols with AOs having 2 to 4 carbon atoms, and adducts of novolak resins with AOs having 2 to 4 carbon atoms. More preferred are aliphatic diols having 2 to 6 carbon atoms, adducts of bisphenols with AOs having 2 to 3 carbon atoms (EO and PO) and adducts of novolak resins with AOs having 2 to 3 carbon atoms (EO and PO).

Among the polycarboxylic acid components, examples of aliphatic (including alicyclic) dicarboxylic acids, aromatic dicarboxylic acids, tri- to hexavalent or higher valent aliphatic (including alicyclic) polycarboxylic acids, and tri- to hexavalent or higher valent aromatic polycarboxylic acids may be the same as those used in the polyester resin (a).

As the polycarboxylic acid component, anhydrides and lower (C1-C4) alkyl esters of these polycarboxylic acids may be used.

Preferred among these polycarboxylic acids are the same as those of the polycarboxylic acid to be used in the polyester resin (a).

The acid value of the polyester resin (B) is preferably 2 to 80, more preferably 5 to 50, and particularly preferably 10 to 30.

The hydroxyl value is preferably 60 or less, more preferably 50 or less, and particularly preferably 5 to 45.

Regarding the molecular weight of the polyester resin (B), Mp is preferably 3000 to 10000, and more preferably 3500 to 9000.

The polyester resin (B) in the present invention can be produced in a similar manner to the production method of conventional polyester. For example, the same method as the production method of the above-mentioned polyester resin (a) can be used.

The polyol component-to-polycarboxylic acid component reaction ratio, as expressed in terms of hydroxyl group-to-carboxyl group equivalent ratio  $[\text{OH}]/[\text{COOH}]$ , is preferably 2/1 to 1/2, more preferably 1.5/1 to 1/1.3, and particularly preferably 1.3/1 to 1/1.2.

The resin for toner of the present invention shows excellent fixing ability even when it is composed solely of a polyester resin (A), but when it contains a polyester (B) together with the polyester resin (A), further improved fixing ability is

obtained. The weight ratio of (A) to (B) is preferably (20 to 100)/(0 to 80), more preferably (30 to 99)/(1 to 70), and particularly preferably (40 to 90)/(10 to 60) where the sum total of (A) and (B) is considered to be 100. When the ratio of the polyester resin (A) is 20 or more, the strength of the resin increases and the fixing ability in a high temperature region is good.

The resin for toner of the present invention is preferably composed solely of a polyester resin (A) or only a polyester resin (A) and polyester resin (B). It, however, may contain another resin unless the characteristic properties of the resin for toner of the present invention are spoiled. The other resin includes, for example, polyester resins other than (A) and (B), vinyl resins [e.g. styrene-alkyl (meth)acrylate copolymers, styrene-diene monomer copolymers], epoxy resins (e.g. ring opening polymerization products of bisphenol A diglycidyl ether, etc.), and urethane resins (e.g. polyaddition products of diol and/or trihydric or higher hydric polyol and diisocyanate, etc.). The Mn of the other resin is preferably 1000 to 1,000,000. The content of the other resin is preferably not more than 10% by weight, and more preferably not more than 5% by weight.

In use of two or more polyester resins combinedly, and in mixing at least one polyester resin with another resin, they may be subjected to powder mixing or melt mixing before-hand or may be mixed at the time of toner compounding.

The temperature in the melt mixing is preferably 80 to 180° C., more preferably 100 to 170° C., and particularly preferably 120 to 160° C.

If the mixing temperature is too low, mixing cannot be accomplished satisfactorily and the system may become inhomogeneous. When the mixing temperature in mixing two or more polyester resins together is excessively high, averaging due to transesterification and other reactions may occur, and it may thus become impossible to maintain those resin properties which are required of toner binders.

The mixing time in melt mixing is preferably 10 seconds to 30 minutes, more preferably 20 seconds to 10 minutes, and particularly preferably 30 seconds to 5 minutes. When the mixing time in mixing two or more polyester resins together is excessively long, averaging due to transesterification and other reactions may occur, and it may thus become impossible to maintain those resin properties which are required of toner binders.

The mixing apparatus for melt mixing includes, for example, batch type mixing apparatus, such as reaction vessels, and continuous mixing apparatus. For attaining uniform mixing at an adequate temperature for a short period of time, a continuous mixing apparatus is preferred. As continuous mixing apparatuses, there are listed extruders, continuous kneaders, three-roll mills and so on. Among them, extruders and continuous kneaders are preferred.

In the case of powder mixing, mixing can be attained using conventional mixing conditions and a conventional mixing apparatus.

Regarding the mixing conditions in powder mixing, the mixing temperature is preferably 0 to 80° C., and more preferably 10 to 60° C. The mixing time is preferably not shorter than 3 minutes, and more preferably 5 to 60 minutes.

The mixing apparatus includes, for example, Henschel mixers, Nauta mixers, and Banbury mixers. Henschel mixers are preferred.

The toner composition of the present invention comprises the resin for toner of the present invention, which serves as a binder resin, a colorant and, according to need, at least one additive selected from mold release agents, charge control agents and fluidizing agents.

As the colorant, any dye, pigment and the like which have been used as a colorant for toner can be used. Specific examples include carbon black, iron black, sudan black SM, fast yellow G, benzidine yellow, pigment yellow, indofast orange, Irgasine red, paranitroaniline red, toluidine red, carmine FB, pigment orange R, lake red 2G, rhodamine FB, rhodamine B lake, methyl violet Blake, phthalocyanine blue, pigment blue, brilliant green, phthalocyanine green, oil yellow GG, Kayaset YG, olasol brown B and oil pink OP. These may be used singly or in combination of two or more of them. According to need, a magnetic powder (a ferromagnetic metal powder such as iron, cobalt and nickel or a compound such as magnetite, hematite and ferrite) may be contained to serve also as a function as a colorant. The content of the colorant is preferably 1 to 40 parts, and more preferably 3 to 10 parts, based on 100 parts of the polyester resin of the present invention. In use of a magnetic powder, the amount thereof is preferably 20 to 150 parts, and more preferably 40 to 120 parts. In the above and following descriptions, "part" means "part by weight".

As the mold release agent, one having a softening point of 50 to 170°C. is preferred. Example thereof includes polyolefin wax, natural wax, aliphatic alcohols having 30 to 50 carbon atoms, fatty acids having 30 to 50 carbon atoms, and their mixtures. Examples of polyolefin wax include (co)polymers of olefins (e.g. ethylene, propylene, 1-butene, isobutylene, 1-hexene, 1-dodecene, 1-octadecene and their mixtures) [including products obtained by (co)polymerization and thermally degraded polyolefin], oxides of olefins (co)polymers prepared by use of oxygen and/or ozone, maleic acid-modified olefin (co)polymers [e.g. products modified with maleic acid or its derivative (maleic anhydride, monomethyl maleate, monobutyl maleate and dimethyl maleate)], copolymers of olefin and unsaturated carboxylic acid [(meth)acrylic acid, itaconic acid, maleic anhydride, etc.] and/or alkyl unsaturated carboxylates [alkyl (meth)acrylates (1 to 18 carbon atoms in the alkyl), alkyl maleates (1 to 18 carbon atoms in the alkyl), etc.], and Sasol wax.

The natural wax includes, for example, carnauba wax, montan wax, paraffin wax and rice wax. An example of the aliphatic alcohols having 30 to 50 carbon atoms is triacontanol. An example of the fatty acids having 30 to 50 carbon atoms is triacontan carboxylic acid.

Examples of the charge control agent include nigrosine dyes, triphenylmethane-based dyes containing a tertiary amine as a side chain, quaternary ammonium salts, polyamine resins, imidazole derivatives, quaternary ammonium salt-containing polymers, metal-containing azo dyes, copper phthalocyanine dyes, metal salts of salicylic acid, boron complexes of benzilic acid, sulfonic acid group-containing polymers, fluorine-containing polymers and halogen-substituted aromatic ring-containing polymers.

The fluidizing agent includes, for examples, colloidal silica, alumina powder, titanium oxide powder and calcium carbonate powder.

Regarding the compositional ratio of the toner composition of the present invention, based on the weight of the toner, the resin for toner of the present invention is preferably 30 to 97% by weight, more preferably 40 to 95% by weight, and particularly preferably 45 to 92% by weight; the colorant is preferably 0.05 to 60% by weight, more preferably 0.1 to 55% by weight, and particularly preferably 0.5 to 50% by weight; among additives, the mold release agent is preferably 0 to 30% by weight, more preferably 0.5 to 20% by weight, and particularly preferably 1 to 10% by weight; the charge control agent is preferably 0 to 20% by weight, more preferably 0.1 to 10% by weight, and particularly preferably 0.5 to 7.5% by

weight; and the fluidizing agent is preferably 0 to 10% by weight, more preferably 0 to 5% by weight, and particularly preferably 0.1 to 4% by weight. The total content of the additives is preferably 3 to 70% by weight, more preferably 4 to 58% by weight, and particularly preferably 5 to 50% by weight. When the compositional ratio of the toner falls within the above-mentioned range, a toner with good electrostatic property can be easily obtained.

The toner composition of the present invention may be prepared by any of conventionally known methods such as a kneading-pulverization method, an emulsion phase-inversion method and a polymerization method. For example, in obtaining of a toner by kneading-pulverization method, it can be prepared by dry blending its components other than a fluidizing agent which are to constitute the toner, melt-kneading, then coarsely pulverizing, finally finely pulverizing using a jet mill pulverizer or the like, further classifying to form fine particles preferably having a volume average particle diameter (D50) of 5 to 20 µm, and then mixing a fluidizing agent. The particle diameter D50 is determined using a Coulter counter [e.g. commercial name: Multisizer III (product of Coulter)].

In preparation of a toner by emulsion phase-inversion method, it can be prepared by dissolving or dispersing in an organic solvent the components other than a fluidizing agent which are to constitute the toner, emulsifying them, for example, by addition of water, and then conducting separation and classification. The volume average particle diameter of the toner is preferably 3 to 15 µm.

The toner composition of the present invention is mixed with carrier particles, such as iron powder, glass beads, nickel powder, ferrite, magnetite, ferrite whose surfaces are coated with a resin (acrylic resin, silicone resin, etc.), depending upon needs, to be used as developer for developing electric latent images.

The weight ratio of toner to carrier particles is usually 1/99 to 100/0. It is also possible to form electric latent images by friction with such a member as a charging blade in lieu of the use of carrier particles.

The toner composition of the present invention is then fixed to a support (e.g. paper and polyester film) by use of a copier, a printer or the like to form a recording material. As a fixing method to a support, conventional heat roll fixing method and flash fixing method, etc. can be used.

## EXAMPLES

Hereinbelow, the present invention will be further described with reference to Examples, by which the present invention is not limited.

A method of measuring properties of polyester resins for toner obtained in examples and comparative examples will be shown in the following.

### 1. Acid Value and Hydroxyl Value

Method Prescribed in JIS K0070 (1992)

In addition, in the case where a sample contained a solvent-insoluble component caused by crosslinking, a sample after melt kneaded in molten state was used in the following method.

Kneading apparatus: Labo plastomill MODEL 4M150 manufactured by Toyo Seiki Seisaku-sho, Ltd.

Kneading conditions: at 130°C., 70 rpm for 30 minutes

### 2. Measurement of Softening Point

A flow tester was used to raise temperature in uniform velocity under the following condition, and a softening point was given by temperature when an amount of the resin outflow reached 1/2.

## 11

Apparatus: Flow Tester CFT-500 manufactured by Shimadzu Corp.

Load: 20 kg

Die: 1 mmφ-1 mm

Rate of temperature rise: 6° C./min

## Example 1

A reaction vessel equipped with a condenser, a stirrer and a nitrogen inlet tube was charged with 950 parts (12.5 mol) of 1,2-propylene glycol (herein after, referred to as propylene glycol), 922 parts (4.8 mol) of dimethyl terephthalate, 37 parts (0.25 mol) of adipic acid and 3 parts of tetrabutoxytitanate as a condensation catalyst, and then a reaction was carried out under a nitrogen stream at 180° C. for 8 hours while methanol produced was distilled off. Subsequently, during a slow increase of the temperature to 230° C., the reaction was carried out under a nitrogen stream for 4 hours while propylene glycol and water produced were distilled off. Thereafter, a further reaction was carried out under a vacuum of 5 to 20 mmHg and the product was taken out when its softening point reached 85° C. The amount of the propylene glycol collected was 521 parts (6.9 mol). The resin taken out was cooled to room temperature and then pulverized to form particles. This is called polyester resin (a1). Polyester resin (a1) had an acid value of 2, a hydroxyl value of 57, an Mn of 2000, and an Mp of 3500.

A reaction vessel equipped with a condenser, a stirrer and a nitrogen inlet tube was charged with 500 parts of polyester resin (a1), 40 parts (0.21 mol) of trimellitic anhydride, and 3 parts of tetrabutoxytitanate as a condensation catalyst. After replacing of the vapor phase in the system by nitrogen, a reaction was carried out at 180° C. under ordinary pressure for 2 hours in a hermetic condition. Thereafter, a further reaction was carried out at 220° C. and a vacuum of 5 to 20 mmHg, and the product was taken out when its softening point reached 180° C. The product was cooled to room temperature and then pulverized to form particles. In the reaction, OH<sub>a</sub>/COOH<sub>b</sub> was 0.81. The product is called polyester resin (A1).

Polyester resin (A1) had an acid value of 17, a hydroxyl value of 2, an Mn of 5200, an Mp of 9400, and a THF-insoluble matter content of 34% by weight.

A reaction vessel equipped with a condenser, a stirrer and a nitrogen inlet tube was charged with 379 parts (1.2 mol) of bisphenol A-EO (2 mol) adduct, 447 parts (1.3 mol) of bisphenol A-PO (2 mol) adduct, 332 parts (2.0 mol) of terephthalic acid and 3 parts of tetrabutoxytitanate as a condensation catalyst, and a reaction was carried out under a nitrogen stream at 230° C. for 5 hours while water produced was distilled off. Subsequently, a further reaction was carried out under a vacuum of 5 to 20 mmHg, followed by cooling to 180° C. when the acid value became 2 or less. Then, 40 parts (0.21 mol) of trimellitic anhydride was added and a reaction was carried out under ordinary pressure for 2 hours in a hermetic condition. The product was taken out, cooled to room temperature and then pulverized to form particles. The product is called polyester resin (B1).

Polyester resin (B1) had an acid value of 21, a hydroxyl value of 37, an Mn of 2000, an Mp of 4200, and a THF-insoluble matter content of 0% by weight.

500 parts of polyester resin (A1) and 500 parts of polyester resin (B1) were melt kneaded in a continuous kneader at a jacket temperature of 150° C. and a residence time of 3 minutes. The melted resin was cooled to room temperature

## 12

and then pulverized by a pulverizer to provide particles. Thus, resin (1) for toner of the present invention was obtained.

## Example 2

5 A reaction vessel equipped with a condenser, a stirrer and a nitrogen inlet tube was charged with 500 parts of polyester resin (a1) obtained in Example 1, 50 parts (0.26 mol) of trimellitic anhydride, and 3 parts of tetrabutoxytitanate as a condensation catalyst. After replacing of the vapor phase in the system by nitrogen, a reaction was carried out at 180° C. under ordinary pressure for 2 hours in a hermetic condition. Thereafter, a further reaction was carried out at 220° C. and a vacuum of 5 to 20 mmHg, and the product was taken out when its softening point reached 160° C. The product was cooled to room temperature and then pulverized to form particles. In the reaction, OH<sub>a</sub>/COOH<sub>b</sub> was 0.65. The product is called polyester resin (A2).

20 Polyester resin (A2) had an acid value of 27, a hydroxyl value of 1, an Mn of 4500, an Mp of 8000, and a THF-insoluble matter content of 20% by weight.

25 500 parts of polyester resin (A2) and 500 parts of polyester resin (B1) given in Example 1 were melt mixed in a continuous kneader at a jacket temperature of 150° C. and a residence time of 3 minutes. The melted resin was cooled to room temperature and then pulverized by a pulverizer to provide particles. Thus, resin (2) for toner of the present invention was obtained.

## Example 3

30 A reaction vessel equipped with a condenser, a stirrer and a nitrogen inlet tube was charged with 950 parts (12.5 mol) of 35 propylene glycol, 158 parts (0.5 mol) of bisphenol A-EO (2 mol) adduct, 824.5 parts (4.3 mol) of dimethyl terephthalate, 109.5 parts (0.75 mol) of adipic acid and 3 parts of tetrabutoxytitanate as a condensation catalyst, and then a reaction was carried out under a nitrogen stream at 180° C. for 8 hours 40 while methanol produced was distilled off. Subsequently, during a slow increase of the temperature to 230° C., the reaction was carried out under a nitrogen stream for 4 hours while propylene glycol and water produced were distilled off. Thereafter, a further reaction was carried out under a vacuum of 5 to 20 mmHg and the product was taken out when its softening point reached 85° C. The amount of the propylene glycol collected was 577.6 parts (7.6 mol). The resin taken out was cooled to room temperature and then pulverized to form particles. This is called polyester resin (a2).

45 50 Polyester resin (a2) had an acid value of 1, a hydroxyl value of 34, an Mn of 3000, and an Mp of 6100.

50 A reaction vessel equipped with a condenser, a stirrer and a nitrogen inlet tube was charged with 500 parts of polyester resin (a2), 30 parts (0.16 mol) of trimellitic anhydride, and 3 parts of tetrabutoxytitanate as a condensation catalyst. After replacing of the vapor phase in the system by nitrogen, a reaction was carried out at 180° C. under ordinary pressure for 2 hours in a hermetic condition. Thereafter, a further reaction was carried out at 220° C. and a vacuum of 5 to 20 mmHg, and the product was taken out when its softening point reached 170° C. The product was cooled to room temperature and then pulverized to form particles. In the reaction, OH<sub>a</sub>/COOH<sub>b</sub> was 0.65. The product is called polyester resin (A3).

55 60 Polyester resin (A3) had an acid value of 18, a hydroxyl value of 2, an Mn of 5000, an Mp of 8700, and a THF-insoluble matter content of 28% by weight.

## 13

500 parts of polyester resin (A3) and 500 parts of polyester resin (B1) given in Example 1 were melt mixed in a continuous kneader at a jacket temperature of 150°C. and a residence time of 3 minutes. The melted resin was cooled to room temperature and then pulverized by a pulverizer to provide particles. Thus, resin (3) for toner of the present invention was obtained.

## Example 4

A pressurizable reaction vessel equipped with a condenser, a stirrer and a nitrogen inlet tube was charged with 1064 parts (14.0 mol) of propylene glycol, 498 parts (3.0 mol) of terephthalic acid, 29 parts (0.2 mol) of adipic acid, and 3 parts of tetrabutoxytitanate as a condensation catalyst. After replacing of the vapor phase in the system by nitrogen, the temperature was increased to 150°C. and then the inside of the system was pressurized with nitrogen to 0.3 MPa. A reaction was carried out at 230°C. for 8 hours while water and propylene glycol produced were distilled off. Then, the pressure in the system was returned to ordinary pressure. Subsequently, a further reaction was carried out at 230°C. while propylene glycol and water produced were distilled off under a vacuum of 5 to 20 mmHg. The product was taken out when its softening point reached 90°C. The amount of the propylene glycol collected was 798 parts (10.5 mol). The resin taken out was cooled to room temperature and then pulverized to form particles. This is called polyester resin (a3).

Polyester resin (a3) had an acid value of 1, a hydroxyl value of 45, an Mn of 2200, and an Mp of 4800.

A reaction vessel equipped with a condenser, a stirrer and a nitrogen inlet tube was charged with 500 parts of polyester resin (a3), 40 parts (0.21 mol) of trimellitic anhydride, and 3 parts of tetrabutoxytitanate as a condensation catalyst. After replacing of the vapor phase in the system by nitrogen, a reaction was carried out at 180°C. under ordinary pressure for 2 hours in a hermetic condition. Thereafter, a further reaction was carried out at 220°C. and a vacuum of 5 to 20 mmHg, and the product was taken out when its softening point reached 170°C. The product was cooled to room temperature and then pulverized to form particles. In the reaction, OHa/COOHb was 0.64. The product is called polyester resin (A4).

Polyester resin (A4) had an acid value of 25, a hydroxyl value of 2, an Mn of 5200, an Mp of 8900, and a THF-insoluble matter content of 24% by weight.

500 parts of polyester resin (A4) and 500 parts of polyester resin (B1) given in Example 1 were melt mixed in a continuous kneader at a jacket temperature of 150°C. and a residence time of 3 minutes. The melted resin was cooled to room temperature and then pulverized by a pulverizer to provide particles. Thus, resin (4) for toner of the present invention was obtained.

## Example 5

The polyester resin (A2) of Example 2 was used as resin (5) for toner of the present invention.

## Comparative Example 1

A reaction vessel equipped with a condenser, a stirrer and a nitrogen inlet tube was charged with 500 parts of polyester resin (a1) given in Example 1, 70 parts (0.36 mol) of trimellitic anhydride, and 3 parts of tetrabutoxytitanate as a condensation catalyst. After replacing of the vapor phase in the system by nitrogen, a reaction was carried out at 180°C.

## 14

under ordinary pressure for 2 hours in a hermetic condition. Thereafter, a further reaction was carried out at 220°C. and a vacuum of 5 to 20 mmHg, but the softening point did not reach 110°C. or higher. Therefore, the product was taken out, cooled to room temperature and then pulverized to form particles.

In the reaction, OHa/COOHb was 0.46. The product is called polyester resin (C1).

10 Polyester resin (C1) had an acid value of 55, a hydroxyl value of 1, an Mn of 2800, an Mp of 3500, and a THF-insoluble matter content of 0% by weight.

15 500 parts of polyester resin (C1) and 500 parts of polyester resin (B1) given in Example 1 were melt mixed in a continuous kneader at a jacket temperature of 150°C. and a residence time of 3 minutes. The melted resin was cooled to room temperature and then pulverized by a pulverizer to provide particles. Thus, resin (6) for toner for comparison use was obtained.

## Comparative Example 2

20 A reaction vessel equipped with a condenser, a stirrer and a nitrogen inlet tube was charged with 500 parts of polyester resin (a1) given in Example 1, 30 parts (0.16 mol) of trimellitic anhydride, and 3 parts of tetrabutoxytitanate as a condensation catalyst. After replacing of the vapor phase in the system by nitrogen, a reaction was carried out at 180°C. under ordinary pressure for 2 hours in a hermetic condition. Thereafter, a further reaction was carried out at 220°C. and a vacuum of 5 to 20 mmHg, and the product was taken out when its softening point reached 180°C. The product was cooled to room temperature and then pulverized to form particles. In the reaction, OHa/COOHb was 1.08. The product is called polyester resin (C2).

25 Polyester resin (C2) had an acid value of 4, a hydroxyl value of 4, an Mn of 4400, an Mp of 7500, and a THF-insoluble matter content of 41% by weight.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9

## 15

was cooled to room temperature and then pulverized to form particles.

This is called polyester resin (a'1).

Polyester resin (a'1) had an acid value of 1, a hydroxyl value of 93, an Mn of 1200, and an Mp of 2500.

A reaction vessel equipped with a condenser, a stirrer and a nitrogen inlet tube was charged with 500 parts of polyester resin (a'1), 70 parts (0.36 mol) of trimellitic anhydride, and 3 parts of tetrabutoxytitanate as a condensation catalyst. After replacing of the vapor phase in the system by nitrogen, a reaction was carried out at 180° C. under ordinary pressure for 2 hours in a hermetic condition. Thereafter, a further reaction was carried out at 220° C. and a vacuum of 5 to 20 mmHg, and the product was taken out when its softening point reached 145° C. The product was cooled to room temperature and then pulverized to form particles. In the reaction, OHa/COOHb was 0.75. The product is called polyester resin (C3).

Polyester resin (C3) had an acid value of 33, a hydroxyl value of 9, an Mn of 2300, an Mp of 4100, and a THF-insoluble matter content of 49% by weight.

500 parts of polyester resin (C3) and 500 parts of polyester resin (B1) given in Example 1 were melt mixed in a continuous kneader at a jacket temperature of 150° C. and a residence time of 3 minutes. The melted resin was cooled to room temperature and then pulverized by a pulverizer to provide particles. Thus, resin (8) for toner for comparison use was obtained.

Examples [6-10], Comparative Examples [4-6]

To each of resins (1) to (5) for toner of the present invention and resins (6) to (8) for toner for comparison use in an amount of 100 parts, 8 parts of carbon black MA-100 (manufactured by Mitsubishi Chemical Co., Inc.), 5 parts of carnauba wax and 1 part of charge control agent T-77 (manufactured by Hodogaya Chemical Co., Ltd.) were added, followed by toner compounding in the following procedures.

Premixing was carried out using a Henschel mixer (FM10B, manufactured by Mitsui Miike Kakoki) and then kneading was carried out using a twin-screw kneader (PCM-30, manufactured by Ikegai Corporation). The mixture was then finely pulverized using a supersonic jet pulverizer [Labojet, product of Nippon Pneumatic Mfg. Co.], followed by classification using an air classifier [model MDS-I, product of Nippon Pneumatic Mfg. Co.] to give toner particles with a particle diameter D50 of 8 µm. Subsequently, 0.5 parts of colloidal silica (aerosil R972: manufactured by Nippon Aerosil Co., Ltd.) was mixed with 100 parts of toner particles using a sample mill to provide toner compositions (T1) to (T5) of the present invention and comparative toner compositions (T6) to (T8).

The results of evaluations made by the following evaluation methods are shown in Table 1.

TABLE 1

| Toner No.              | MFT<br>(° C.) | HOT<br>(° C.) | Anti-blocking<br>property | Pulverisability<br>µm |
|------------------------|---------------|---------------|---------------------------|-----------------------|
| Toner composition (T1) | 125           | 230           | ⊕                         | 12                    |
| Toner composition (T2) | 120           | 230           | ⊕                         | 11                    |
| Toner composition (T3) | 120           | 230           | ⊕                         | 12                    |
| Toner composition (T4) | 125           | 230           | ⊕                         | 12                    |

## 16

TABLE 1-continued

| Toner No.                             | MFT<br>(° C.) | HOT<br>(° C.) | Anti-blocking<br>property | Pulverisability<br>µm |
|---------------------------------------|---------------|---------------|---------------------------|-----------------------|
| 5 Toner composition (T5)              | 120           | 230           | ⊕                         | 11                    |
| Comparative toner composition (T6)    | 120           | 190           | Δ                         | 11                    |
| Comparative toner composition (T7)    | 135           | 230           | ⊕                         | 15                    |
| 10 Comparative toner composition (T8) | 140           | 220           | ○                         | 13                    |

## [Method of Evaluation]

## [1] Minimum Fixing Temperature (MFT)

15 A fixing device of a commercially available copier (AR5030: manufactured by Sharp Corporation) was used to evaluate a non-fixing image developed by the copier. A fixing roll temperature, at which a image density remaining percentage after rubbing of a fixed image by a pad became at least 70%, was made a minimum fixing temperature.

## [2] Hot Offset Occurrence Temperature (HOT)

20 Like the above MFT, evaluation of fixing was made, and the existence of hot offset on a fixed image was evaluated visually. A fixing roll temperature, at which hot offset was occurred, was made an hot offset occurrence temperature.

## [3] Test of Toner's Anti-blocking Property

25 Each of the toner compositions was conditioned in a high-temperature and high-humidity environment (50° C., 85% R.H.) for 48 hours. Under the same environment the blocking state of each developer was visually judged, and the image quality of a copy produced by use of a commercially available copier (AR5030; produced by Sharp Corp.) was also observed.

## Criterion

30 ○: No blocking of the toner is recognized and image quality after 3000-sheet copying is good.

○: No blocking of the toner is recognized, but slight disorder in image quality after 3000-sheet copying is recognized.

40 A: Blocking of the toner is visually recognized and disorder in image quality after 3000-sheet copying is recognized.

x: Blocking of the toner is visually recognized and images are no longer formed before 3000-sheet copying.

## [4] Pulverisability

45 A coarsely ground toner which had been kneaded in a twin-screw kneader and cooled, which could pass through 8.6 mesh but remain on 30 mesh, was finely pulverized using a supersonic jet pulverizer "Labojet", product of Nippon Pneumatic Mfg. Co.

Pulverising pressure: 0.5 MPa

Adjuster ring: 15 mm

Size of a louver: medium

Pulverising time: 10 minutes

50 The resultant was subjected, without classification, to volume average particle diameter measurement using a Coulter counter TAII (produced by Coulter Electronics, Ltd., U.S.A.). This test was considered as a test of pulverisability. In this measuring method, it can be said that when the volume average particle diameter is 12 µm or less, the pulverisability is good.

## INDUSTRIAL APPLICABILITY

55 The toner composition and the resin for toner of the present invention are useful as a toner for developing electrostatic charge images and a resin for such toner which are excellent in low-temperature fixing ability and hot offset resistance.

## 17

The invention claimed is:

1. A resin for toner, the resin comprising a polyester resin (A) produced by reacting a polyester resin (a) having an acid value of 6 mgKOH/g or less and a hydroxyl value of 10 to 80 mgKOH/g with at least one carboxylic acid (b) selected from the group consisting of aliphatic carboxylic acids, aromatic carboxylic acids, their anhydrides and lower alkyl (C1-C4) esters, wherein the equivalent ratio OH<sub>a</sub>/COOH<sub>b</sub> is 0.55 to 1.0 where OH<sub>a</sub> represents the equivalent of the hydroxyl groups originating in (a) in the reaction of (a) and (b) and COOH<sub>b</sub> represents the equivalent of the carboxyl groups originating in (b) in the reaction of (a) and (b), wherein the polyester resin (A) has an acid value of 13 to 50 mgKOH/g and a hydroxyl value of 8 mgKOH/g or less, and wherein 30 to 100 mol % of the polyol component constituting the polyester resin (A) is an aliphatic diol having 2 to 6 carbon atoms.

2. The resin for toner according to claim 1, wherein the carboxylic acid (b) is a divalent or higher valent aromatic carboxylic acid.

3. The resin for toner according to claim 2, wherein the polyester resin (A) has a THF-insoluble matters in a content of 1 to 50% by weight.

4. The resin for toner according to claim 3, wherein the resin contains, together with the polyester resin (A), a polyester resin (B) other than the (A) which is free from any THF-insoluble matter.

5. The resin for toner according to claim 2, wherein the resin contains, together with the polyester resin (A), a polyester resin (B) other than the (A) which is free from any THF-insoluble matter.

6. The resin for toner according to claim 1, wherein the polyester resin (A) has a THF-insoluble matters in a content of 1 to 50% by weight.

30

## 18

7. The resin for toner according to claim 6, wherein the resin contains, together with the polyester resin (A), a polyester resin (B) other than the (A) which is free from any THF-insoluble matter.

5 8. The resin for toner according to claim 1, wherein the resin contains, together with the polyester resin (A), a polyester resin (B) other than the (A) which is free from any THF-insoluble matter.

10 9. A toner composition comprising the resin for toner according to claim 1, a colorant and, if necessary, one or more additives selected from mold release agents, charge control agents and fluidizing agents.

15 10. A resin for toner, the resin comprising a polyester resin (A') which has an acid value of 13 to 50 mgKOH/g and a hydroxyl value of 8 mgKOH/g or less and has a THF-insoluble matter in a content of 1 to 50% by weight, wherein 30 to 100 mol % of the polyol component constituting the (A') is an aliphatic diol having 2 to 6 carbon atoms and the carboxylic acid component constituting the (A') comprises a trivalent or higher valent aromatic polycarboxylic acid.

20 11. The resin for toner according to claim 10, wherein the resin contains, together with the polyester resin (A), a polyester resin (B) other than the (A) which is free from any THF-insoluble matter.

25 12. A toner composition comprising the resin for toner according to claim 10, a colorant and, if necessary, one or more additives selected from mold release agents, charge control agents and fluidizing agents.

\* \* \* \* \*